

1

2,836,566

## CLEANING COMPOSITION AND METHOD

Ira J. Duncan, Detroit, Mich., assignor to Detrex Chemical Industries, Inc., a corporation of Michigan

No Drawing. Application January 27, 1954  
Serial No. 406,595

3 Claims. (Cl. 252—137)

This invention relates to a composition and a method of cleaning metal objects, and more particularly concerns an alkali cleaning solution containing a corrosion inhibitor for cleaning carbonized and grease-carbon incrustations from metal objects containing tin, without corroding the tin. More particularly, the invention relates to a composition and method wherein a strong alkaline cleaning solution is applied to one or more bread-baking pans wherein at least two unlike metals or metal oxides may be immersed in a common solution without any substantial corrosion of either metal or oxide.

The cleaning of badly soiled tin bakery pans without damage to the tin surface has long presented a problem. Such pans are usually cleaned in hot solutions of alkaline cleaners consisting of alkali metal salts of silicates, phosphates, carbonates, borates, etc., together with suitable tin inhibitors. Well known inhibitors are the alkali metal salts of chromates, dichromates and silicates. Even with these inhibitors, complete protection to the tin surface is not always possible, especially at a pH above about 12. Cleaners of a pH below about 12 have less tendency to attack the tin surface, but their cleaning is usually slow which makes it necessary to boil the pans for many hours to effect cleaning.

Some pans used in the bread-baking industry are made of tin coated steel and have reinforcing bands constructed of heavier tin coated steel or galvanized steel. Recently, aluminized steel bands have been used by the pan manufacturers on tin coated steel pans. Such pans are usually subjected to a heat treatment of about 425° F. for several hours prior to being used. In the opinion of the trade, superior baking characteristics are thus obtained. This treatment gives to the pans a grayish blue color, commonly referred to as "burn-in," or tin oxide coating. Accordingly the pans may have tin or tin oxide surfaces, while the straps may have tin, tin oxide, aluminum, or aluminum oxide surfaces. Bread pans constructed of both tin plated steel and aluminized steel bands present an even more difficult cleaning problem, since the presence of these unlike metals causes an increased tendency for galvanic cell activity to occur, which results in severe tin attack.

When two different metals are brought into contact with the cleaning solution an electro-chemical phenomenon is involved. In the case of tin coated steel pans bearing an oxide film and covered with carbonized grease and other bakery soils, there is a reducing action on the oxide coating. Thereby, numerous small areas of the oxide film are often removed which exposes the pure metal to the solution at these points. The more noble metal oxide and the pure metal in contact with the cleaning solution tend to set up a galvanic cell action. Also, when two metals, e. g., tin and aluminum, are in contact with a common cleaning solution there is a tendency for both tin and aluminum to go into solution. When this takes place the metals become electro-negative. Since the solution potential of tin and aluminum are not of the same magnitude there is set up a galvanic action between

2

the two metals. Pans constructed of both tin and aluminum and covered with bakery soil might exhibit an even greater galvanic action than similar clean pans.

The function of silicate or chromate inhibitors is to 5 passivate the metal surface and thus prevent the oxide from being removed and to prevent the galvanic cell activity. This is sometimes difficult to accomplish completely with certain types of bakery soil and with certain types of pans. Galvanic cell activity as outlined above 10 interferes with the inhibiting action of chromate or silicate inhibitors.

It is accordingly an object of this invention to provide 15 a composition and method which overcome the foregoing difficulties and disadvantages. Another object is to provide a method of cleaning carbonized and grease-carbon incrustations from baking containers having surfaces containing at least two materials selected from the group consisting of tin, aluminum, tin oxide, and aluminum oxide, without any substantial attack on the surface. Another 20 object is to provide a corrosion inhibitor for strong alkali cleaner compositions of this character which is effective at pH values in excess of 11.8, even in the presence of two or more unlike metals or metal oxides. Other objects and advantages of the invention will appear in 25 further detail hereinafter.

For cleaning the type of bread pans described above I have discovered a new inhibitor for use in alkaline cleaners which prevents attack on the tin surface even at a pH of 12 or higher. The inhibited composition consists of 30 an alkaline solution containing the copper-amine complex ion.

The copper-amine complexion may be made by combining a water soluble copper salt with an organic amino compound. A wide variety of water soluble copper salts 35 are suitable for the practice of this invention, including cupric sulfate, cupric chloride, cupric acetate, cuprous chloride and cuprous cyanide. There is also a wide selection of mono- or poly-amino organic compounds which 40 coat with the copper ion in accordance with this invention, including 1,3-diamino butane; monethanolamine, 2-amino, 2-methyl, propanol-1; "Polyamine T" (distillation residues from the distillation of amines, sold by Carbide and Carbon Chemical Corp., New York); "CSC-38" (distillation residues from the distillation of hydroxy amines, sold by Commercial Solvents Corp., Terre Haute, Indiana). Also, several synthetic detergents of the 45 amino condensation type were shown to be effective. Examples of the latter are the "Ninols" manufactured by the Ninol Laboratories of Chicago, Ill., which are amides formed by the reaction between fatty acids and alkanol amines.

The above list of copper salts and organic amino compounds is merely illustrative of the types of compounds which protect tin pans in alkaline solutions, and is not intended to be exhaustive. Any compatible combination of copper salt and organic amino compound may be utilized provided the copper salt is water soluble producing a copper ion which reacts with the amine, and provided the amino compound includes a water-soluble amino (NH<sub>2</sub>) group. Soluble compounds, such as NH<sub>4</sub>OH, 50 are not suitable.

If desired, the inhibitor may be mixed as a copper-amine complex. However equally good results are obtained by mixing together the alkaline components, the copper salt and the amino compound. The latter method is more convenient from the manufacturing standpoint. It is emphasized that the presence of both the copper ion and the amino compound is necessary in order to protect the metal surface in accordance with this invention.

The preferred range of proportions for a mixture of solid ingredients is about 75-93% by weight strong alkali cleaning chemicals such as alkali metal silicates,

carbonates, phosphates, borates, hydroxides and the like, about 2-10% by weight water soluble copper salt and about 5-15% by weight organic amino compound. In solution, the copper amine complex ion is formed, and this should be present in a proportion of approximately 3-15% by weight based on the total weight of copper amine and complex plus alkali cleaning chemicals, the weight of the complex being calculated on an additive Cu and amino group ( $\text{NH}_2$ ) basis.

Typical cleaning compositions containing copper salts and amines which effectively clean tin-aluminum pans in a common solution without attack to the metal surfaces appear below.

|                     | Percent |
|---------------------|---------|
| Sodium metasilicate | 20-50   |
| Trisodium phosphate | 0-25    |
| Soluble copper salt | 3-10    |
| Amino compound      | 4-15    |
| Soda ash            | 0-63    |

The above ranges of percentage composition are preferred ranges, but are not to be taken as setting out the limits of effectiveness of this invention.

The following specific examples further illustrate preferred compositions and methods in accordance with this invention:

*Example 1*

A composition was prepared consisting of:

|                                               | Pounds |
|-----------------------------------------------|--------|
| Sodium metasilicate                           | 50     |
| Sodium carbonate                              | 35     |
| Polyamine T (amino acid distillation residue) | 10     |
| Cupric chloride                               | 5      |

The above composition was dissolved in water at a concentration of 4.5 ounces per gallon. Strips of burned-in tin were immersed in the solution at boiling temperature for several hours and, upon removing the strips, it was observed that the tin was not visibly attacked.

It has been disclosed in U. S. Patent No. 2,050,122 to W. Reuss et al. that the cobaltic amine ion is an effective corrosion-preventing agent for tin when added to certain alkaline cleaning compositions. However, when this agent was tested in cleaning compositions for cleaning combination tin and aluminum bread pans protection was not obtained, resulting in severe attack on the tin surface.

*Example 2*

A composition was prepared consisting of:

|                                               | Pounds |
|-----------------------------------------------|--------|
| Sodium metasilicate                           | 50     |
| Sodium carbonate                              | 35     |
| Polyamine T (amino acid distillation residue) | 10     |
| Cobaltic chloride                             | 5      |

The above composition was dissolved in water at a concentration of 4.5 ounces per gallon. Strips of burned-in tin were brightened within 15 minutes when placed in the solution at boiling temperature.

*Example 3*

The procedure of Example 1 was repeated, substituting equal amounts of cupric sulfate and cupric acetate for copper chloride, and in each instance substantially identical results were observed.

*Example 4*

A mixture was prepared consisting, by weight, of:

|                     | Percent |
|---------------------|---------|
| Sodium metasilicate | 48      |
| Sodium chromate     | 10      |
| Soda ash            | 30      |
| Cupric sulfate      | 2       |
| Polyamine T         | 10      |

This mixture, dissolved as in Example 1, was effective for cleaning baked-in tin pans having aluminized steel bands, and did not visibly corrode the tin or aluminized steel even after immersion for three hours.

*Example 5*

Another mixture, specified below, was tested as in Example 4, with substantially identical results:

|                        | Percent |
|------------------------|---------|
| 10 Sodium metasilicate | 35      |
| Sodium chromate        | 10      |
| Cupric sulfate         | 2       |
| Polyamine T            | 8       |
| Sodium bicarbonate     | 20      |
| 15 Soda ash            | 25      |

*Example 6*

|                                                                                                       |    |
|-------------------------------------------------------------------------------------------------------|----|
|                                                                                                       | 50 |
| Sodium metasilicate                                                                                   | 50 |
| Soda ash                                                                                              | 38 |
| 20 Cupric sulfate                                                                                     | 5  |
| Mixed amino hydroxy compounds (amino acid distillation residue supplied by Commercial Solvents Corp.) | 7  |

*Example 7*

|                                                                                                          |    |
|----------------------------------------------------------------------------------------------------------|----|
|                                                                                                          | 50 |
| Sodium metasilicate                                                                                      | 50 |
| Soda ash                                                                                                 | 39 |
| Cupric sulfate                                                                                           | 5  |
| 30 Mixed amino hydroxy compounds (amino acid distillation residue supplied by Commercial Solvents Corp.) | 6  |

*Example 8*

|                              |    |
|------------------------------|----|
|                              | 25 |
| 35 Sodium metasilicate       | 25 |
| Tri sodium phosphate         | 25 |
| Soda ash                     | 39 |
| Copper sulfate               | 5  |
| Mixed amino hydroxy compound | 6  |

*Example 9*

|                     |    |
|---------------------|----|
|                     | 50 |
| Sodium metasilicate | 50 |
| Soda ash            | 35 |
| Polyamine T         | 10 |
| 45 Cupric chloride  | 5  |

Burned-in tin strips, placed in a boiling solution of each of these mixtures at 4 to 5 ounces per gallon, were not attacked after several hours. With similar procedure, the same results were obtained in Examples 10-13.

*Example 10*

|                        | Percent |
|------------------------|---------|
| 55 Sodium metasilicate | 50      |
| Soda ash               | 35      |
| Polyamine T            | 10      |
| Cuprous chloride       | 5       |

*Example 11*

|                        |    |
|------------------------|----|
|                        | 50 |
| 60 Sodium metasilicate | 50 |
| Soda ash               | 35 |
| Polyamine T            | 10 |
| Cuprous cyanide        | 5  |

*Example 12*

|                     |    |
|---------------------|----|
|                     | 50 |
| Sodium metasilicate | 50 |
| Soda ash            | 35 |
| Polyamine T         | 10 |
| Cuprous acetate     | 5  |

*Example 13*

|                     |    |
|---------------------|----|
|                     | 50 |
| Sodium metasilicate | 50 |
| Soda ash            | 35 |
| Polyamine T         | 10 |
| Cupric sulfate      | 5  |

## Example 14

|                     |    |
|---------------------|----|
| Sodium metasilicate | 50 |
| Soda ash            | 39 |
| Copper sulfate      | 5  |
| 1,3-diamino butane  | 6  |

The above chemicals were dissolved in water in an amount to produce a concentration of 4 to 5 ounces per gallon. At boiling temperature, even after several hours immersion, burned-in tin strips were not substantially attacked.

The same procedure was followed, producing the same results, substituting the mixtures of Examples 15-17 which follow:

## Example 15

## Percent

|                     |    |
|---------------------|----|
| Sodium metasilicate | 50 |
| Soda ash            | 39 |
| Copper sulfate      | 5  |
| Monoethanolamine    | 6  |

## Example 16

|                             |    |
|-----------------------------|----|
| Sodium metasilicate         | 50 |
| Soda ash                    | 39 |
| Copper sulfate              | 5  |
| 2-amino 2-methyl 1-propanol | 6  |

## Example 17

|                                                                   |    |
|-------------------------------------------------------------------|----|
| Sodium metasilicate                                               | 50 |
| Soda ash                                                          | 39 |
| Copper sulfate                                                    | 5  |
| "Ninol" amino condensate product (mixed fatty acid alkanol-amine) | 6  |

## Example 18

## Pounds

|                 |    |
|-----------------|----|
| Soda ash        | 75 |
| Triethanolamine | 15 |
| Cuprous sulfate | 10 |

## Example 19

|                             |    |
|-----------------------------|----|
| Soda ash                    | 55 |
| Trisodium phosphate         | 20 |
| 2-amino 2-methyl 1-propanol | 15 |
| Cupric acetate              | 10 |

## Example 20

|                    |    |
|--------------------|----|
| Sodium tetraborate | 20 |
| Soda ash           | 75 |
| Monoethanolamine   | 10 |
| Cuprous chloride   | 5  |

which method said object is immersed in a strong hot aqueous alkali cleaner solution having a pH above about 11.8 in the presence of a dissimilar surface selected from the group consisting of tin, aluminum and their oxides, 5 which solution tends to attack the surface of said work object by galvanic corrosive action, the novel step which comprises immersing said work object in a solution consisting essentially of water and about four to five ounces per gallon of a solute consisting essentially of about 10 20-50% by weight alkali metal metasilicate, 3-10% water-soluble copper salt selected from the group consisting of sulfate, chloride, acetate and cyanide, and about 4-15% by weight amine selected from the group consisting of 1,3-diamino butane, monoethanolamine, 2-amino-2-methyl 1-propanol and triethanolamine, and about 25-63% by weight soda ash.

2. An alkaline cleaning solution for removing bakery incrustations from baking containers, said solution having a pH above about 11.8 and consisting essentially of water and about 4 to five ounces per gallon of solute consisting essentially of about 20-50% by weight alkali metal metasilicate, 3-10% water-soluble copper salt selected from the group consisting of sulfate, chloride, acetate, and cyanide and, about 4-15% by weight amine selected from the group consisting of 1,3-diamino butane, monoethanolamine, 2-amino-2-methyl 1-propanol and thiethanolamine, and about 25-63% by weight soda ash, the percentages being based upon the total weight of said alkali metal metasilicate, soda ash, copper salt, and amine.

3. An alkaline metal cleaning composition for removing bakery incrustations from bakery containers consisting essentially by weight of about 50% sodium metasilicate, 39% soda ash, 5% copper sulfate, and 6% monoethanolamine.

## References Cited in the file of this patent

## UNITED STATES PATENTS

|    |           |               |               |
|----|-----------|---------------|---------------|
| 40 | 2,050,122 | Reuss et al.  | Aug. 4, 1936  |
|    | 2,168,909 | Mason         | Aug. 8, 1939  |
| 20 | 2,377,966 | Reed          | June 12, 1945 |
| 15 | 2,525,079 | Reeder et al. | Oct. 10, 1950 |
| 10 | 2,706,180 | Sylvester     | Apr. 12, 1955 |
| 45 | 2,731,420 | Sylvester     | Jan. 17, 1956 |

## FOREIGN PATENTS

|         |               |               |
|---------|---------------|---------------|
| 661,370 | Great Britain | Nov. 21, 1951 |
|---------|---------------|---------------|

## OTHER REFERENCES

Sequestrene, pp. 5, 9, 27, pub. by Geigy Industrial Chemicals, New York (1952).

Synthetic Detergents by McCutcheon, p. 405, pub. by 55 MacNair Dorland, New York (1950).

Having thus described my invention, I claim:

1. In a method of removing bakery deposits from a work object having a surface selected from the group which includes tin and aluminum and their oxides without appreciably attacking any of said tin, aluminum or oxides, in

UNITED STATES PATENT OFFICE  
CERTIFICATE OF CORRECTION

Patent No. 2,836,566

May 27, 1958

Ira J. Duncan

It is hereby certified that error appears in the printed specification of the above numbered patent requiring correction and that the said Letters Patent should read as corrected below.

Column 1, line 39, for "indusy" read -- industry --; line 69, for "aluminum" read -- aluminum --; column 2, line 52, for "hopper" read -- copper --; column 3, line 7, strike out "and"; line 57, for "ounches" read -- ounces --; column 6, line 27, for "thieethanolamine" read -- tri-ethanolamine --.

Signed and sealed this 21st day of October 1958.

(SEAL)

Attest:

KARL H. AXLINE  
Attesting Officer

ROBERT C. WATSON  
Commissioner of Patents